



US006782590B2

(12) **United States Patent**  
Rock et al.

(10) Patent No.: **US 6,782,590 B2**  
(45) Date of Patent: **Aug. 31, 2004**

(54) **VELOUR FABRIC ARTICLES HAVING FLAME RETARDANCE AND IMPROVED DYNAMIC INSULATION PERFORMANCE**

(75) Inventors: **Moshe Rock**, Brookline, MA (US); **Edward P. Dionne**, Sanford, ME (US); **Charles Haryslak**, Haverhill, MA (US); **William K. Lie**, Methuen, MA (US); **Douglas Lumb**, Methuen, MA (US); **Jane Hunter**, Londonderry, NH (US)

(73) Assignee: **Maiden Mills Industries, Inc.**, Lawrence, MA (US)

(\*) Notice: Subject to any disclaimer, the term of this patent is extended or adjusted under 35 U.S.C. 154(b) by 0 days.

(21) Appl. No.: **10/683,773**

(22) Filed: **Oct. 10, 2003**

(65) **Prior Publication Data**

US 2004/0083768 A1 May 6, 2004

**Related U.S. Application Data**

(62) Division of application No. 10/122,024, filed on Apr. 12, 2002, which is a continuation-in-part of application No. 09/982,720, filed on Oct. 18, 2001, which is a continuation-in-part of application No. 09/883,643, filed on Jun. 18, 2001, now abandoned, which is a division of application No. 09/347,825, filed on Jul. 2, 1999, now abandoned.

(51) **Int. Cl. 7** ..... **D04H 5/02**

(52) **U.S. Cl.** ..... **28/105; 66/194**

(58) **Field of Search** ..... **28/103-115, 140, 28/159-162, 167, 168; 66/191, 194; 442/136, 311-312, 306-308**

(56) **References Cited**

**U.S. PATENT DOCUMENTS**

3,837,943 A \* 9/1974 Ploch et al. ..... 156/93  
4,067,209 A 1/1978 Kucera et al.  
4,103,518 A \* 8/1978 Lombardi et al. ..... 66/107

|             |          |                       |
|-------------|----------|-----------------------|
| 4,546,026 A | 10/1985  | Kowalski              |
| 5,520,022 A | * 5/1996 | Callaway ..... 66/194 |
| 5,557,950 A | 9/1996   | Richards              |
| 5,598,615 A | 2/1997   | Takada                |
| 6,082,147 A | 7/2000   | Rock et al.           |
| 6,164,095 A | 12/2000  | Rock et al.           |

**FOREIGN PATENT DOCUMENTS**

|    |           |         |
|----|-----------|---------|
| EP | 0 111 409 | 6/1984  |
| FR | 2 313 486 | 12/1976 |
| FR | 2 512 081 | 3/1983  |
| FR | 2 747 133 | 10/1997 |
| GB | 2 106 153 | 7/1983  |

**OTHER PUBLICATIONS**

International Search Report; EP 03 25 2366; Sep. 2003; P. Van Gelder.

Patent Abstracts of Japan; vol. 1998, No. 03, Feb. 27, 1998; JP 09 302560; Nov. 25, 1997.

\* cited by examiner

Primary Examiner—Danny Worrell

(74) Attorney, Agent, or Firm—Fish & Richardson P.C.

(57) **ABSTRACT**

A velour fabric article consists of a fabric body having a technical face formed by a filament stitch yarn and a technical back formed by a loop yarn. The filament stitch yarn includes a heat sensitive material, e.g. a hot melt material or a heat shrinkable material, and/or an elastomeric material, such as spandex. The loop yarn includes flame retardant material, such as M-Aramid fiber. The fabric body has a velour surface formed at one or both of the technical back and the technical face. Raised fibers of at least one of the technical face and the technical back may be entangled, including in and/or through interstices of the fabric body, toward the other of the technical face and the technical back, e.g., by a hydroentanglement process applied after finishing. The fabric body has permeability of about 90 ft<sup>3</sup>/ft<sup>2</sup>/min, or less, under a pressure difference of  $\frac{1}{2}$  inch of water across the fabric body.

**15 Claims, 6 Drawing Sheets**





FIG. 1



FIG. 2

PRIOR ART  
FIG. 3

FIG. 12



FIG. 13



FIG. 4





FIG. 14





## VELOUR FABRIC ARTICLES HAVING FLAME RETARDANCE AND IMPROVED DYNAMIC INSULATION PERFORMANCE

This application is a division of the U.S. application Ser. No. 10/122,024 filed Apr. 12, 2002, which is a continuation-in-part of U.S. application Ser. No. 09/982,720, filed Oct. 18, 2001, now pending, which is a continuation-in-part of U.S. application Ser. No. 09/883,643, filed Jun. 18, 2001, now abandoned, which is a division of U.S. application Ser. No. 09/347,825, filed Jul. 2, 1999, now abandoned, the entire disclosures of all of which are incorporated herein by reference.

This invention relates to velour fabric articles, and, more particularly, to velour fabric articles having improved dynamic insulation performance due to relatively greater densification and tortuosity, and improved flame retardance.

### BACKGROUND

Velour fabric articles having one or more fleece or raised surface regions at one surface or at both surfaces, e.g., achieved by processes of sanding, brushing and/or napping of exposed fibers, are known to have good insulation performance under static conditions, i.e., in calm or still air with no wind blowing through the fabric. However, the insulating performance of these fabric articles drops rapidly under dynamic conditions, i.e., in a chilling wind. As a result, a consumer wearing a velour fabric article will often find it necessary to also wear a shell, e.g., of woven nylon or other low permeability material, when conditions are likely to be windy.

It is also known to increase the thermal insulation performance of velour fabric articles by incorporating a relatively coarser stitch yarn and/or by tightening the stitch. However, these approaches result in fabric articles with very poor stretch, increased stiffness and increased weight.

### SUMMARY

According to one aspect of the invention, a double-face velour fabric article comprises a fabric body having a technical face formed by a filament stitch yarn and a technical back formed by a loop yarn, the filament stitch yarn comprising heat sensitive material and the loop yarn comprising flame retardant material, the fabric body having a velour surface formed at one or both of the technical back and the technical face, and the heat sensitive material responding to application of heat during processing to increase tortuosity with a result of the fabric body having permeability of about 90 ft<sup>3</sup>/ft<sup>2</sup>/min or less under a pressure difference of  $\frac{1}{2}$  inch of water across the fabric body (according to the testing method of ASTM Designation: D 737-96, "Standard Test Method for Air Permeability of Textile Fabrics," the entire disclosure of which is incorporated herein by reference).

Preferred embodiments of this aspect of the invention may include one or more of the following additional features. The flame retardant material comprises m-Aramid fibers. The heat sensitive material is preferably selected from the group consisting of polypropylene, polyester, and polyamide. The heat sensitive material comprises heat shrinkable material, preferably selected from the group consisting of polypropylene, nylon, and polyester. The heat sensitive material responds to application of dry heat and/or to application of wet heat, e.g. steam or hot water, e.g. at about 212° F. to about 450° F. applied for about 2 minutes to about 60 minutes. The filament stitch yarn comprises elastomeric

material, e.g. spandex. Filaments of the heat sensitive material and filaments of the elastomeric material are commingled or plaited together. The filament stitch yarn is a cored yarn comprising a core and a sheath, the sheath comprising hot melt material. The core material is preferably selected from the group consisting of polyester and nylon, and the hot melt material is preferably selected from the group consisting of polypropylene, polyester and polyamide. The loop yarn is split, e.g. by application of heat, e.g. the loop yarn of fine denier fibers or filaments comprises an "islands-in-sea" construction, or by application of a chemical, e.g. caustic soda, or by mechanical action, e.g. napping, to release multiple small diameter filaments. The loop yarn and/or the filament stitch yarn are textured. Raised fibers of the velour surface, of at least one of the technical face and the technical back, are entangled, including in and/or through interstices of the fabric body toward the other of the technical face and the technical back. Raised fibers of the technical back are entangled, including in and/or through interstices of the fabric body, toward the technical face. The fabric body has a velour surface region formed at the technical back or the fabric body has a velour surface region formed at each of the technical back and the technical face.

According to another aspect of the invention, a double-face velour fabric article comprises a fabric body having a technical face formed by a filament stitch yarn and a technical back formed by a filament loop yarn or spun loop yarn, the filament stitch yarn comprising elastomeric material and the loop yarn comprising flame retardant material, the fabric body having a velour surface formed at one or both of the technical back and the technical face, and the fabric body having permeability of about 90 ft<sup>3</sup>/ft<sup>2</sup>/min or less under a pressure difference of  $\frac{1}{2}$  inch of water across the fabric body.

Preferred embodiments of both of these aspects of the invention may include one or more of the following additional features. The flame retardant material comprises m-Aramid fibers. The elastomeric material comprises spandex. The fabric body has permeability of about 70 ft<sup>3</sup>/ft<sup>2</sup>/min or less. Raised fibers of the velour surface of at least one of the technical face and the technical back is entangled, including in and/or through interstices of the fabric body toward the other of the technical face and the technical back. Preferably, raised fibers of the technical back are entangled, including in and/or through interstices of the fabric body, toward the technical face.

According to yet another aspect of the invention, a method of forming a velour fabric body comprises the steps of: joining a filament or spun loop yarn and a filament stitch yarn to form a fabric prebody, the filament stitch yarn forming a technical face of the fabric prebody and the loop yarn forming a technical back of the fabric prebody, the filament stitch yarn comprising heat sensitive material and the loop yarn comprising flame retardant material, finishing at least one of the technical face and the technical back of the fabric prebody, thereby to form a velour fabric body having at least one velour surface region, entangling raised fibers of at least one of the technical face and the technical back, including in and/or through interstices of the fabric body, thereby to increase density and tortuosity of the fiber body, the fabric body having permeability of about 90 ft<sup>3</sup>/ft<sup>2</sup>/min or less under a pressure difference of  $\frac{1}{2}$  inch of water across the fabric body.

Preferred embodiments of this aspect of the invention may include one or more of the following additional features. The method comprises the further step of entangling the raised fibers in a process of hydroentanglement, by

directing fine, high-pressure jets upon at least one of the technical face and the technical back. The method comprises the further step of directing fine, high-pressure jets upon the technical back, to cause raised fibers of the velour surface of the technical back to entangle, including in and/or through interstices of the fabric body, toward the technical face. The filament stitch yarn comprises heat sensitive material, and the method comprises the further step of exposing said fabric body to heating sufficient to cause a response by the heat sensitive material, thereby to increase tortuosity. The method comprises the further step of entangling the raised fibers in a process of hydroentanglement, by directing fine, high-pressure water jets upon at least one of the technical face and the technical back. The method comprises the further step of directing fine, high pressure jets (e.g., water jets or air jets) upon the technical back, to cause raised fibers of the velour surface of the technical back to entangle, including in and/or through interstices of the fabric body, toward the technical face. The method comprises the step of finishing the technical face and the technical back of the fabric prebody, thereby to form a velour fabric body having velour regions at opposite surfaces. The method comprises exposing the fabric body to the heating sufficient to cause a response by the heat sensitive material during dyeing and/or during finishing. The method comprises exposing the fabric body to dry heat and/or to wet heat, e.g., steam or hot water. The method comprises exposing the fabric body to heating sufficient to cause a response by the heat sensitive material for about 2 minutes to about 60 minutes at about 212° F. to about 450° F. The method comprises exposing the fabric body to heating sufficient to cause a response by the heat sensitive material, thereby to increase tortuosity with a result of the fabric body having permeability of about 70 ft<sup>3</sup>/ft<sup>2</sup>/min or less. The method comprises joining a loop yarn and a filament stitch yarn, the filament stitch yarn comprising elastomeric material, e.g., spandex.

An objective of the invention is to provide velour fabric articles having flame retardance and improved dynamic insulation performance while avoiding increased weight and/or loss of stretch and/or loss of flexibility. A further objective is to provide velour fabric articles that may be worn in chilling, windy conditions without markedly diminished insulation performance. Generally, tortuosity, and therefore density, is increased by using heat-sensitive and/or elastomeric materials in the stitch yarns and entangling the loop yarn fibers. The improved dynamic insulation performance achieved in conditions of relative wind speed (i.e., wind blowing and/or movement of the wearer in relation to ambient atmosphere) enhances flame retardance properties by allowing less air to penetrate through the fabric construction. Thus flame retardance is enhanced, e.g. in accordance with very stringent flame retardance requirements of the protective cloth and military markets, e.g., as set forth in NFPA 1975-94 (the complete disclosure of which is incorporated herein by reference), by including fibers of inherent flame retardant material, e.g., m-Aramid fibers (NOMEX®, as available from E. I. du Pont de Nemours and Company, of Wilmington, Del.) in the loop yarn of fleece or raised surface regions of the resulting velour fabric articles.

The details of one or more embodiments of the invention are set forth in the accompanying drawings and the description below. Other features, objects, and advantages of the invention will be apparent from the description and drawings, and from the claims.

#### DESCRIPTION OF DRAWINGS

FIG. 1 is a somewhat diagrammatic end section view of a double-face fabric prebody, e.g., as formed in a reverse plaiting circular knitting process.

FIG. 2 is a somewhat diagrammatic end section view of a double-face velour fabric article of the invention formed by finishing the double-face fabric prebody of FIG. 1; and

FIG. 3 is a somewhat diagrammatic end section view of a prior art double-face velour fabric article that is comparable to the double-face velour fabric article of FIG. 2.

FIG. 4 is a perspective view of a segment of a circular knitting machine, and FIGS. 5-11 are sequential views of a cylinder latch needle in a reverse plaiting circular knitting process, e.g., for use in forming the double-face fabric prebody of FIG. 1.

FIG. 12 is a somewhat diagrammatic end section view of a double-face velour fabric article being subjected to a process of hydroentanglement; and

FIG. 13 is a similar, somewhat diagrammatic end section view of a resulting double-face velour fabric article of the invention, having improved dynamic insulation performance.

FIG. 14 is a plot of curves showing the relationship between change in effective thermal insulation and wind velocity for covers or fabrics of different permeability (P. Larose, "The Effect of Wind on the Thermal Resistance of Clothing with Special Reference to the Protection Given by Coverall Fabrics of Various Permeabilities," Canadian Journal of Research, Vol. 25, Sec. A, No. 4, (July 1947), pp. 169-190.).

FIGS. 15-20 are somewhat diagrammatic end section views of other embodiments of double-face velour fabric articles of the invention formed of filament stitch yarns and/or loop yarns including or consisting largely of materials with characteristics selected for improving dynamic insulation performance of the fabric article, namely heat sensitive materials, elastic materials and/or combinations thereof;

FIG. 21 is a somewhat diagrammatic end section view of an alternative embodiment of a double-face velour fabric article of the invention formed of loop yarns including, or consisting largely of, materials with characteristics selected for improving flame retardance; and

FIG. 22 is a somewhat diagrammatic end section view of another alternative embodiment of a velour fabric article of the invention having raised or fleece surface region(s) formed at a single surface by finishing fibers of loop yarns including, or consisting largely of, materials with characteristics selected for improving flame retardance.

Like reference symbols in the various drawings indicate like elements.

#### DETAILED DESCRIPTION

Referring to FIG. 1, a double-face fabric prebody 12, e.g., for use in forming a double-face velour fabric article 10 of the invention (FIG. 2), is formed by joining a stitch yarn 14 and a loop yarn 16 in a standard reverse plaiting circular knitting (terry knitting) process (see FIGS. 4-11), e.g., as described in *Knitting Technology*, by David J. Spencer (Woodhead Publishing Limited, 2nd edition, 1996), the entire disclosure of which is incorporated herein by reference. In the terry knitting process, the stitch yarn 14 forms the technical face 18 of the resulting fabric prebody 12 and the loop yarn 16 forms the opposite technical back 20, where it is formed into loops 22. In the fabric prebody 12 formed by reverse plaiting circular knitting, the loop yarn 16 extends outwardly to overlie and cover the stitch yarn 14 at the technical face 18.

The loop yarn 16 forming the technical back 20 of the knit fabric body 12 can be made of any synthetic or natural

material. The cross section and luster of the fibers or filaments may be varied, e.g., as dictated by requirements of the intended end use. The loop yarn 16 can be a textured or flat filament or, preferably, a yarn of fine denier filaments or fibers (e.g., 1.5 dpf or lower), with a textured yarn being preferred for relatively greater dynamic insulating effect, as discussed below. The loop yarn overall denier is typically in the range of about 70 denier to 300 denier, with a preferred count of about 150 denier. At the preferred count, the filament count range is from about 100 filaments to 300 filaments, therefore providing a denier per filament (dpf) of from 1.5 to 0.5, respectively. A relatively smaller dpf, e.g. 1 dpf, is preferred for relatively greater dynamic insulating effect, as will be discussed below. A preferred commercial loop yarn is a 150/132 denier textured polyester yarn of fine denier filaments or fibers with a dpf of 1.14, e.g. as available from UNIFI, Inc., of Greensboro, N.C.

The stitch yarn 14 forming the technical face 16 of the knit fabric body 12 can be also made of any type of synthetic or natural material in a textured or flat filament yarn, with a textured yarn being preferred for relatively greater dynamic insulating effect. The range of stitch yarn count denier is typically between about 50 denier to 150 denier. Where the loop yarn is 150/132 textured, the preferred stitch yarn count is about 100 denier, and the filament count ranges from about 34 filaments to 200 filaments, i.e. 100/34 to 100/200, resulting in dpf from about 3 dpf to 0.5 dpf, with relatively finer filaments being preferred, again, for relatively greater dynamic insulating performance. A preferred stitch yarn is 100/136 denier textured polyester with about 0.7 dpf, e.g. as available commercially from UNIFI, Inc. Another preferred yarn is 130/408 denier textured polyester with about 0.3 dpf, e.g. as available from Hyosung, Inc., of Seoul, Korea.

From these examples, it can be seen that, for achieving markedly improved dynamic insulating performance, use of a textured 150/132 loop yarn and a textured 100/136 stitch 35 yarn is preferred.

In comparison, in a prior art double-face velour fabric article (100, FIG. 3) without the improved dynamic insulation performance of the present invention, a typical stitch 40 yarn 102 is 70/34 denier filament textured polyester, with individual fiber fineness of greater than 2.0 dpf, e.g. as available commercially from UNIFI, Inc.

In a preferred method of the invention, the fabric prebody 12 is formed by reverse plaiting on a fine cut circular knitting machine (e.g., 28 cut). This is principally a terry knit construction, where segments 22 of the loop yarn 16 cover the stitch yarn 14 on the technical face 18 and loops 23 of the loop yarn 16 form loops 23 at the technical back 20 of the fabric prebody 12 (see FIG. 1).

The fabric prebody 12 is next subjected to finishing. During the finishing process, the technical face and technical back surfaces 18, 20, respectively, of the fabric prebody 12, with the segments 22 of loop yarn 16 overlying the stitch 45 yarn 14 at the technical face surface 18 and the loops 23 formed at the technical back surface 20, go through a finishing process such as sanding, brushing and/or napping, to generate a velour 24, 26. The yarn fibers are raised at both faces of the fabric prebody 12 (FIG. 1), including the technical face 18 and the technical back 20, to form the velour 24, 26 at each face of the fabric body 30 of the double-face velour fabric article 10 (FIG. 2) of the invention. The fabric prebody 12 and/or fabric body 10 may also be treated, e.g., chemically, to make it hydrophobic.

Referring to FIG. 12, after finishing, the fabric article 10 is next subjected to a process of hydroentanglement, such as

employed in fabrication of spun staples yarn and in the fabrication of non-woven fabrics. During this process, fine, high-pressure water jets 32 (or air jets) are directed onto, e.g., the technical back 20 of the fabric article 10. In this 5 manner, raised fibers 34 of the velour surface of the technical back 20 are entangled, including in and/or through interstices of the fabric body 30, toward the technical face 18. The hydroentanglement process thus serves to densify the velour surface, resulting in the double-face fabric article 40 (FIG. 13), advantageously, without substantial increase in 10 bulk or thickness, for improved dynamic insulation, i.e. against through-flow of air, e.g., in a chilling wind. By way of example only, after finishing, the technical back 20 of a double-face velour fabric article 10 may be treated by 15 hydroentanglement using fine, high-pressure water jets 32, e.g., with water applied at 100 m/sec to 350 m/sec through jets having apertures of 0.01 mm to 1.0 mm diameter. Alternatively, raised fibers of the technical face may be 20 entangled in and/or through interstices of the fabric body, toward the technical back.

Entangling raised fibers of the technical back, i.e., of the loop yarn, including in and/or through interstices of the fabric body, toward the technical face, results in relatively 25 greater densification and therefore greater tortuosity, e.g., as compared to entanglement of raised fibers of the technical face, including in and/or through interstices of the fabric body, toward the technical back. Entangling from back to face, in addition to resulting in a relatively greater increase 30 in tortuosity, also increases smoothness of the fabric/garment outer surface, while entangling from face to back increases tortuosity and increases smoothness of the fabric/garment inner surface.

Fabric performance and aesthetics of the fabric article 40 can also be adjusted by selection of knitting gauge (e.g., in 35 the range of about 18 to about 36, and preferably about 28), yarn type (e.g., preferably textured, or flat filament), yarn denier (e.g., about 70 to about 300, and preferably about 100), fiber denier (e.g., about 0.3 to about 1.5, and preferably about 1.0), etc. Adjustment of jet speed and/or aperture size, 40 e.g., within the ranges mentioned above, can further or instead be employed to adjust fabric performance and/or aesthetics.

The fabric article 40 is thereafter heat set to stabilize the 45 fabric article width.

In this and other embodiments of the invention described below, heat may be applied to the fabric body, e.g. dry heat and/or wet heat, such as hot water or steam, e.g. during 50 finishing or dyeing. As mentioned elsewhere, the stitch yarn (and/or the loop yarn) may include heat sensitive and/or elastomeric materials.

In a resulting double-face velour fabric article 10 of this embodiment of the invention, the overall density, i.e., weight per length, of the filament stitch yarn 14 is closely comparable 55 to stitch yarn 102 used in a comparable prior art fabric article 100 having velour 104, 106 at the opposite faces. The diameter of the filament stitch yarn 14 may be slightly greater than that of the prior art stitch yarn 102 (likely due to increased filament-to-filament engagement of the filaments of the filament stitch yarn 14). The yarn count and gauge of the double-face velour fabric article 10 of the invention are also substantially the same as those for the comparable prior art fabric article 100. As a result, the weight and stretch performance of the double-face velour 60 fabric article 10 of the invention is closely comparable to the weight and stretch of the prior art double-face velour fabric article 100 of the same gauge and yarn count.

The fact that the weight density of the filament stitch yarn 14 and the stitch yarn 102 are the same indicates that the ratio of yarn material to open volume for each of the respective articles is also approximately the same. However, in the filament stitch yarn 14, and in the resulting double-face velour fabric article 10 of the invention, the average cross sectional area of the individual filaments is considerably less than the average cross sectional area of filaments in the stitch yarn 102 employed in the comparable prior art fabric article 100, e.g. the denier per filament (dpf) of the preferred filament stitch yarn 14 is about 0.7 dpf, as compared to 3.0 dpf for the stitch yarn 102 of comparable prior art fabric article 100. As a result, the paths for passage of air, e.g., a chilling wind, through double-face velour fabric article 10 of the invention, while relatively more numerous, are also considerably smaller and relatively more tortuous, as compared to a comparable prior art double-face velour fabric article 100. The enhanced performance of the fabric article of the invention is achieved by increasing the yarn count and the filament count to make the paths through the fabric more tortuous, thus making it more difficult for air, i.e., a chilling wind, to penetrate quickly through the double-face velour fabric article 10 of the invention. As a result, the dynamic insulation performance of the double-face velour fabric of the invention is dramatically increased over the prior art.

In FIG. 14, there is reproduced a plot of curves showing the relationship between change in effective thermal insulation and wind velocity for covers or fabrics of different permeabilities, as appeared in an article by P. Larose, entitled "The Effect of Wind on the Thermal Resistance of Clothing with Special Reference to the Protection Given by Coverall Fabrics of Various Permeabilities," which appeared in Canadian Journal of Research (Vol. 25, Sec. A, No. 4, (July 1947), pp. 169-190), the entire disclosure of which is incorporated herein by reference. The permeabilities of the materials tested varied between 0 and 193 ft<sup>3</sup>/ft<sup>2</sup>/min under a pressure difference of  $\frac{1}{2}$  inch of water across the fabric.

In particular, it can be seen in the plot that at zero wind velocity there is relatively little difference in insulating performance among the materials tested. The dynamic insulating performance for each of the materials tested also decreased with increasing wind velocity. However, as may be seen in the plot, the rate of decrease in dynamic insulating performance was much more precipitous in fabrics of relatively greater permeability, i.e. as permeability increased, the rate of loss of dynamic insulating performance with increasing wind velocity was relatively smaller for fabrics of low permeability, as compared to fabrics having relatively greater permeability.

In Table A (below), the improvement in dynamic insulation performance of double-face velour fabric articles 10 (FIG. 2) of the invention in a chilling wind can easily be seen when compared to the performance of a comparable prior art double-face velour fabric article 100 (FIG. 3). In particular, the double-face velour fabric article 10 of the invention has considerably better dynamic insulating performance, and good static (no wind) and dynamic (windy) insulation performance, due to the increased tortuosity of air paths through the fabric, with good stretch properties and light weight.

The word "tortuosity" is used to describe the fabric property enhanced according to this invention by increasing yarn count and filament count. The paths through the fabric are made more "tortuous" than those of prior art fabrics, and greater "tortuosity" results in greater dynamic insulating effect. In addition, if a given fabric body is subjected to less

than normal stretching, resulting in reduced final width of the fabric (i.e., the width resulting after heat setting of the fabric during the finishing process), the higher, still, the dynamic insulating performance of the resulting fabric article of the invention.

TABLE A

|                                           | A1                                                                                             | A2                  | B1                  | B2                  |
|-------------------------------------------|------------------------------------------------------------------------------------------------|---------------------|---------------------|---------------------|
| 10 Loop Yarn                              | 150/100<br>textured                                                                            | 150/132<br>textured | 150/100<br>textured | 150/132<br>textured |
| Stitch Yarn                               | 100/34<br>textured                                                                             | 100/34<br>textured  | 100/34<br>textured  | 100/34<br>textured  |
| Width                                     | 58-inch<br>cuttable                                                                            | 58-inch<br>cuttable | 54-inch<br>cuttable | 54-inch<br>cuttable |
| 15 "Dynamic<br>Insulating<br>Performance" | 100-110 cfm                                                                                    | 60-70 cfm           | 70-80 cfm           | 50-60 cfm           |
| 20 Compare: A1 to A2                      | A2 has finer loop yarn, and therefore relatively better dynamic insulating performance.        |                     |                     |                     |
| 20 Compare: A1 to B1                      | B1 has narrower width, and therefore better dynamic insulating performance.                    |                     |                     |                     |
| 20 Compare: A1 to B2                      | B2 has finer loop yarn, and therefore better dynamic insulating performance.                   |                     |                     |                     |
| 20 Compare: A1 to B2                      | B2 has finer loop yarn and narrower width, and therefore better dynamic insulating performance |                     |                     |                     |

In other preferred embodiments, fabric articles of the invention having relatively greater densification and tortuosity, and therefore increased dynamic insulation performance for enhanced protection from wind penetration, are achieved by incorporation of stitch yarns and/or loop yarns of predetermined selected characteristics. For example, stitch yarns and/or loop yarns including, or formed largely of, heat sensitive materials, e.g. hot melt or heat shrinkable materials, and/or elastomeric materials, such as spandex, may be employed.

For example, referring now to FIG. 15, in a preferred embodiment, a fabric article 30 of the invention formed by reverse plaiting on a fine cut circular knitting machine includes a stitch yarn 32 and a loop yarn 34 finished into a velour 36, 38 at the opposite surfaces. The stitch yarn 32 includes, or consists largely of, yarn or filaments of heat sensitive material 33, e.g. heat shrinkable material, or hot melt material (typically commingled (e.g., blended) with other fiber that will maintain yarn integrity after heat treatment). The loop yarn 34, which, in this embodiment, may be a filament yarn but is more typically a spun yarn, includes, or consists largely of, fibers of suitable flame retardant material, e.g., such as m-Aramid, 1.5 denier, e.g. as manufactured by E. I. du Pont de Nemours and Company, of Wilmington, Del., under the trademark NOMEX®. The m-aramide fibers may be used alone, or in a blend, e.g. with fibers of p-aramide, e.g. as manufactured by E. I. du Pont de Nemours and Company, of Wilmington, Del., under the trademark KEVLAR®, and/or with fibers of other suitable material having good electrostatic dissipation characteristics. Suitable heat sensitive materials include polypropylene, nylon, polyester, polyamide, and the like, preferably with high shrinkage, e.g., about 5% to about 50% after about 2 minutes to about 60 minutes at about 212° F. to about 450° F. Heat is thereafter applied to the fabric article, e.g., dry heat and/or wet heat, such as hot water or steam, e.g. during dyeing and/or finishing. Upon exposure to heat, the hot melt material fuses to narrow or fill interstices between the yarns filaments, and the heat shrinkable material shortens and thickens, and/or reduces in effective length, thus to reduce the paths for passage of chilling wind through the fabric and thereby increase the tortuosity and the dynamic insulation performance of the fabric article 30 of the invention.

Referring next to FIG. 16, in another embodiment, in a fabric article 40 of the invention, the stitch yarn 42 comprises a cored yarn 43 having a core formed, e.g., of polyester or nylon, with a sheath formed of a heat sensitive material, e.g., a hot melt material, such as polypropylene, polyester or nylon, e.g. as available commercially from Engineered Yarn Company, of Fall River, Mass. The loop yarn 44 includes, or consists largely of, fibers of flame retardant material 46. During heating of the fabric article of this embodiment, e.g. during dyeing and/or finishing, the hot melt material of the sheath fuses, thus increasing the tortuosity and further reducing the paths for passage of chilling wind through the fabric and improving the dynamic insulation performance of the fabric article 40 of the invention.

Referring now to FIG. 17, in a fabric article 50 of the invention, the stitch yarn 52 includes elastomeric material 53, e.g. such as spandex. The loop yarn 54 includes, or consists largely of, fibers of flame retardant material 56. The elastomeric material 53 in the stitch yarn 52 also provides for relatively greater densification and tortuosity, and therefore increased dynamic insulation performance for enhanced protection from wind penetration, as well as providing for fabric stretch and enhanced wearer comfort.

Referring now to FIG. 18, a fabric article 60 of the invention may also be formed of stitch yams 62 including or consisting largely of combinations of heat sensitive materials 63 and elastomeric materials 65. For example, stitch yams employed in the fabric article 60 may include fibers or filaments of different characteristics that have been commingled or plaited together. The loop yarn 64 includes, or consists largely of, fibers of flame retardant materials 66.

Referring to FIG. 19, in another embodiment, a fabric article 70 of the invention is formed of loop yarns 72 of standard denier that, upon application of heat, e.g. during dyeing and/or finishing, split axially into multiple, elongated fibers or filaments. The result is a reduction or narrowing of paths for passage of chilling wind through the fabric, to increase tortuosity and dynamic insulation performance of the fabric article 70. The loop yarns may be caused to split also by application, e.g., of a chemical treatment, e.g. caustic soda, or by application of a mechanical action, e.g. napping.

Referring finally to FIG. 20, in yet another embodiment, a fabric article 80 of the invention is formed of loop yarns 82 having an "islands-in-sea" construction. Namely, the loop yarns 82 are formed of a hot melt polymeric body ("sea") containing multiple filaments ("islands") of small diameter, e.g. 0.01 to 0.03 denier. Upon application of heat to the fabric article 80, e.g., during dyeing and/or finishing, the hot melt material melts to release the individual, small diameter filaments. Again, the release of the small filaments results in increased tortuosity and dynamic insulation performance of the fabric article 80.

Alternatively, referring to FIG. 21, in a different embodiment, a double face velour fabric article 90 of the invention is formed of very bulky filament stitch yarn 92 with relatively low shrinkage. The resulting fabric article 90 will be significantly heavier, less drapeable, and will have relatively poor stretch/recovery, e.g. as compared to the embodiments described above. However, the high bulk, high thickness of the raised surface regions 94, 96 formed by finishing fibers of the loop yarn 93 of flame retardant material 98 will provide enhanced protection or shielding of the stitch yarn 92 from excessive heat and thermal shrinkage, as well as from burning and melting.

Finally, referring to FIG. 22, in yet another embodiment of the invention, a velour fabric article 100, in this case

having one or more raised or fleece surface regions 102 at only one surface, is formed with a plaiting circular knit construction from a loop yarn 104, e.g. including, or consisting largely of, flame retardant material 106, such as m-Aramid fibers (NOMEX®) of 1.5 denier, and a filament stitch yarn 108, e.g. including, or consisting largely of, thermoplastic filament yarn 110, formed of materials such as polyester, nylon, or polypropylene, commingled or plaited with spandex material 112, such as LYCRA® (also available from E. I. du Pont). The fibers of the loop yarn 104 are finished at the technical back 114 to create a velour or fleece region 102 at one surface. The fabric article 100 of this embodiment has good stretch, when tested according to ASTM 2594, in both length and width dimensions. The single face velour fabric 100 can be formed into articles for tight fit, which enhances the comfort and insulation performance in dynamic (windy) conditions. Positioning the fleece surface 102 of flame retardant material 106 against the wearer's skin also shields against potential drip of the thermoplastic stitch yarn material 110 onto the skin, e.g. in a fire condition. Positioning of the flame retardant surface region 102 against the skin also improves thermal insulation (in cold weather), as well as providing enhanced thermal insulation, as measured on a Frazier air permeability unit in accordance with ASTM D-737. It also shields against penetration of material from melting fibers of the stitch yarn 108 through to burn the wearer's skin.

Due to the increased tortuosity, including after heat treatment, a fabric article of the invention formed with stitch yarns including or consisting largely of heat sensitive materials and/or elastomeric materials, such as spandex, and/or loop yarns formed of heat sensitive materials and/or elastomeric materials such as spandex, and/or cored yarns having a sheath of hot melt material, have enhanced dynamic insulation performance, e.g. as compared to a prior art fabric article 100 (FIG. 3) having the same weight. As a result, the fabric articles of the invention are particularly suited for use, e.g., in lightweight clothing and the like for use in extreme conditions of chilling wind and cold temperature.

Examples of fabric articles of the invention formed with heat sensitive materials and/or elastomeric materials will now be described. The air permeability was tested according to ASTM D-737 (the complete disclosure of which is incorporated herein by reference) on a Frazier machine with  $\frac{1}{2}$  of water pressure drop.

#### EXAMPLE 1

A fabric article of the invention, designated S/7380, was formed of a stitch yarn consisting of 150/34 POWER-STRETCH™ heat shrinkable textured polyester, available from UNIFI, Inc., and a loop yarn consisting of 150/132 textured polyester. After exposure to heat, the air permeability of the finished fabric article was 70 ft<sup>3</sup>/ft<sup>2</sup>/min.

#### EXAMPLE 2

Another fabric article of the invention, designated E555P, was formed of a stitch yarn consisting of 50/36 textured polyester with 20 denier spandex on every other end plaited with the 50/36 textured polyester and a loop yarn consisting of 150/132 textured polyester. After exposure to heat, the air permeability of the finished fabric article was 59 ft<sup>3</sup>/ft<sup>2</sup>/min.

#### EXAMPLE 3

Yet another fabric article of the invention, designated E657Y, was formed of a stitch yarn consisting of 50/36 textured polyester commingled with 40/20 textured polypro-

## 11

pylene and a loop yarn consisting of 100/96 textured polyester. After exposure to heat, the air permeability of the finished fabric article was 38–40 ft<sup>3</sup>/ft<sup>2</sup>/min.

## EXAMPLE 4

Another fabric article of the invention, designated E667Q, was formed of a stitch yarn consisting of 100/34 POWER-STRETCH™ heat shrinkable textured polyester and a loop yarn consisting of 100/96 textured polyester. After exposure to heat, the air permeability of the finished fabric article was 60–70 ft<sup>3</sup>/ft<sup>2</sup>/min.

A number of embodiments of the invention have been described. Nevertheless, it will be understood that various modifications may be made without departing from the spirit and scope of the invention. For example, any suitable type of yarn may be employed. Also, other suitable methods of constructing a velour fabric article of the invention may be employed. For example, in the preferred embodiment described above, the construction provided by reverse plaiting is employed in order to expose the loop yarn 16 for finishing at both surfaces of the fabric body, with segments 22 of the loop yarn 16 overlaying the stitch yarn 14 at the technical face 18 and formed into loops 23 at the technical back 20. This is preferred, for reasons of dynamic insulation performance, over a construction in which only the loop yarn is finished. However, where improvement of dynamic insulation performance is not the primary or an overwhelming consideration, a construction exposing the stitch yarn and the loop yarn side by side for finishing at one or both surfaces of a fabric body may be preferred. In embodiments of fabric articles of the invention formed with heat sensitive materials, heat may be applied other than or in addition to during dyeing and/or finishing, e.g., before, after, or between these stages of manufacture. Also, referring again to FIG. 13, a double-face velour fabric article 40 of the invention may be formed by applying the hydroentanglement process to the technical face 18 and/or the technical back 20, e.g., using fine, high-pressure water jets 32 and/or 32', respectively.

As mentioned above, a fabric article with stitch yarn and/or loop yarn comprising heat sensitive and/or elastomeric material may also be entangled or hydroentangled according to the invention.

Accordingly, other embodiments are within the scope of the following claims.

What is claimed is:

1. A method of forming a velour fabric body, said method comprising the steps of: joining a loop yarn and a filament stitch yarn to form a fabric prebody, the filament stitch yarn forming a technical face of the fabric prebody and the loop yarn forming a technical back of the fabric prebody, the filament stitch yarn comprising heat sensitive material and the loop yarn comprising flame retardant material,

finishing at least one of said technical face and said technical back of the fabric prebody, thereby to form a velour fabric body having at least one velour surface region, and entangling raised fibers of at least one of the technical face and the technical back, including in and/or through interstices of the fabric body, thereby to

## 12

increase density and tortuosity of the fiber body, the fabric body having permeability of about 90 ft<sup>3</sup>/ft<sup>2</sup>/min or less under a pressure difference of  $\frac{1}{2}$  inch of water across the fabric body.

- 5 2. The method of forming a velour fabric body of claim 1, comprising the further step of entangling the raised fibers in a process of hydroentanglement, by directing fine, high pressure jets upon at least one of the technical face and the technical back.
- 10 3. The method of forming a velour fabric body of claim 1 or claim 2, comprising the further step of directing fine, high pressure jets upon the technical back, to cause raised fibers of the velour surface of the technical back to entangle, including in and/or through interstices of the fabric body, 15 toward the technical face.
- 15 4. The method of forming a velour fabric body of claim 1, wherein the filament stitch yarn comprises heat sensitive material, and said method comprises the further step of exposing said fabric body to heating sufficient to cause a 20 response by the heat sensitive material, thereby to increase tortuosity.
- 20 5. The method of forming a velour fabric body of claim 1, wherein said method comprises the step of finishing said technical face and said technical back of the fabric prebody, 25 thereby to form a velour fabric body having velour regions at opposite surfaces.
- 25 6. The method of forming a velour fabric body of claim 1, comprising exposing said fabric body to said heating sufficient to cause a response by said heat sensitive material 30 during dyeing.
- 30 7. The method of forming a velour fabric body of claim 1, comprising exposing said fabric body to said heating sufficient to cause a response by said heat sensitive material during finishing.
- 35 8. The method of forming a velour fabric body of claim 1, comprising exposing said fabric body to dry heat.
- 35 9. The method of forming a velour fabric body of claim 1, comprising exposing said fabric body to wet heat.
- 40 10. The method of forming a velour fabric body of claim 9, comprising exposing said fabric body to steam.
- 40 11. The method of forming a velour fabric body of claim 9, comprising exposing said fabric body to hot water.
- 45 12. The method of forming a velour fabric body of claim 9, comprising exposing said fabric body to said heating sufficient to cause a response by said heat sensitive material for about 2 minutes to about 60 minutes at about 212° F. to about 450° F.
- 45 13. The method of forming a velour fabric body of claim 9, comprising joining a loop yarn and a filament stitch yarn, 50 the filament stitch yarn comprising elastomeric material.
- 50 14. The method of forming a velour fabric body of claim 9, comprising exposing said fabric body to heating sufficient to cause a response by said heat sensitive material, thereby to increase tortuosity with a result of said fabric body having permeability of about 70 ft<sup>3</sup>/ft<sup>2</sup>/min or less.
- 55 15. The method of forming a velour fabric body of claim 9, wherein the filament stitch yarn comprises elastomeric material.

\* \* \* \* \*